

## UNITED STATES PATENT OFFICE

MARSDEN H. HUNT, OF EAST PITTSBURGH, PENNSYLVANIA, ASSIGNOR TO WESTINGHOUSE ELECTRIC & MANUFACTURING COMPANY, A CORPORATION OF PENNSYLVANIA

## RESISTOR MATERIAL AND METHOD OF MAKING THE SAME

Application filed November 1, 1922. Serial No. 598,420.

This invention relates to resistor materials, more particularly to high-resistance materials and to methods of manufacturing the same.

It is among the objects of this invention to provide a resistor material which shall be simple and economical to manufacture and which may be baked at a low temperature for a short time to increase the efficiency of the process.

In practising my invention, I provide a resistor material of any suitable type but, preferably, comprising a mixture of a conducting substance, such as lamp-black, conducting oxides or the like, an inert non-conducting material, such as powdered quartz, clay or any suitable powdered rock, and a binder consisting of a glass or an enamel which has a low fusing point and which may be soluble or insoluble in the fused state.

Preferably, I employ a mixture of powdered glass 35 parts, powdered quartz 52 parts, clay 10 parts and lamp-black 3 parts.

The proportions of ingredients may be varied according to the resistance desired, the mechanical strength and the size and the shape of the article in which it is to be incorporated.

My material may be prepared as follows: The above-specified ingredients are measured in the correct proportions and thoroughly mixed either in the dry state, wherein the materials are ground together and passed through fine-mesh screens a suitable number of times to facilitate mixing, or by a wet process in which the ingredients are ground together with sufficient liquid to allow thorough mixing of the same and subsequent drying to the proper consistency for shaping the resistor body.

I may utilize a plastic, pliable mass of resistor material and extrude it through dies of suitable shape or a mixture, in a fluid state, containing water and a suitable electrolyte, such as carbonate or silicate of sodium, and cast such fluid mixture into molds of plaster of Paris which absorb the water, thus providing bodies of the desired form.

The formed bodies are dried, generally at a temperature above 150° C. The dried bodies are then fired or baked in either an oxidizing or a reducing atmosphere. The temperature and time of firing depend upon the properties desired in the finished product, but generally the temperature used is between 500° C. and 900° C. for a short period of time, varying from five to twenty minutes.

My process of making resistor material is characterized by the use of a low-fusing-point flux or glass which allows the firing of the material at a relatively low temperature in a short time under any suitable conditions of atmosphere. The result of this procedure is a baked article which is strongly bonded together by means of the low-fusing-temperature flux.

I am aware that it has been proposed to provide resistor materials consisting of metallic oxides, clay, quartz and fieldspar by making a suitable mixture of said materials, and firing the same at a high temperature, thereby producing a vitreous, non-porous body. My invention differs from the above in that I use a low temperature and complete the baking operation in a comparatively short time, the resultant material being non-vitreous and porous.

My invention has a further advantage in that trial pieces may be made from a mixture and quickly baked and tested, whereby the plastic mixture may be modified by the addition of the proper material, if the proportions of ingredients are found to be incorrect. This reduces the manufacturing losses which have hitherto occurred with materials of this kind. The low temperature and the short time period of baking lower the cost of production and increase the production for a given capacity of furnace, the life of which is increased because of its operation at a temperature which is not injurious or destructive.

I claim as my invention:

1. A resistor material comprising a silicate glass, quartz, clay and lampblack, partially fused and bonded together.
2. A resistor material comprising a sili-

100

cate glass 35 parts, quartz 52 parts, clay 10 parts and lampblack 3 parts.

3. The method of preparing resistor material which comprises providing a mixture of conducting and non-conducting substances and a low-temperature fusing glass having a fusion temperature below 900° C., intimately mixing said substances with an inorganic plastic silicate and then firing the same at a temperature below 900° C. to partially fuse and bind the ingredients together.

4. The method of preparing resistor material which comprises providing a mixture of conducting and non-conducting substances and a low-temperature fusing glass having a fusion temperature below 900° C., intimately mixing said substances with an inorganic plastic silicate and then firing the same at a temperature of 500° to 900° C. to partially fuse and bind the ingredients together.

5. The method of preparing resistor material which comprises providing a mixture of conducting and non-conducting substances and a low-temperature fusing glass having a fusion temperature below 900° C., intimately mixing said substances with an inorganic plastic silicate and then firing the same at a temperature of 500° to 900° C. for a sufficient length of time to partially fuse and bind the ingredients together.

6. A method of preparing resistor material which comprises providing a mixture of conducting and non-conducting substances, a plastic clay and a silicate glass that fuses at a temperature below 900° C. and firing the same at a temperature below 900° C. for a time period of from five to twenty minutes, to partially fuse and bind the ingredients together.

7. A method of preparing resistor material which comprises providing a mixture of conducting and non-conducting substances, a plastic clay and a silicate glass that fuses at a low-temperature and firing the same at a temperature of 500° C. to 900° C. for a period of between five and twenty minutes, to partially fuse and bind the ingredients together.

8. A method of preparing resistor material which comprises forming a mixture of a silicate glass, quartz, clay and lampblack and firing the same at 500° to 900° C.

55 9. A method of preparing resistor material which comprises forming a mixture of glass, quartz, clay and lampblack and firing the same at a temperature of 500° C. to 900° C. for a period of between five and twenty minutes.

10. A resistor material comprising a fluxing glass having a fusion temperature below 900° C., quartz, clay and lampblack, the fluxing glass being present in sufficient proportions so that the material may be

fused and bound together at a temperature of 500 to 900° C.

11. A resistor material comprising quartz and lampblack in the proportions of about 14 parts quartz, one part lampblack, sufficient clay so that the mixture may be readily molded, and a sufficient quantity of a fluxing glass having a fusion temperature below 900° C. so that the mixture may be fired at a temperature of between 500 and 900° C.

12. A method of preparing resistor material which comprises grinding a mixture of a conducting and non-conducting substance, a plastic clay and a silicate glass that fuses at a temperature below 900° C. thoroughly together and firing the same at a temperature below 900° C. to partially fuse and bind the ingredients together.

13. A method of preparing resistor material which comprises grinding a mixture of a conducting and non-conducting substance, a plastic clay and a silicate glass that fuses at a temperature below 900° C. thoroughly together, forming the mass into the shape of a resistor, drying the formed body at a temperature of about 150° C. and then firing the dried body at a temperature between 500 and 900° C.

In testimony whereof, I have hereunto subscribed my name this 27th day of October, 1922.

MARSDEN H. HUNT.

100

105

110

115

120

125

130